

## UNITED STATES PATENT OFFICE

2,228,309

## PROPELLENT POWDER

Ellsworth S. Goodyear, Kenil, N. J., assignor to  
Hercules Powder Company, Wilmington, Del., a  
corporation of Delaware

No Drawing. Application December 13, 1939,  
Serial No. 309,041

7 Claims. (Cl. 52—13)

This invention relates to an improved propellant powder for ordnance field pieces, and more particularly to a propellant powder which is smokeless, flashless and non-hygroscopic.

5 The ordnance art for many years used black powder in all field pieces and were severely hampered because black powder produced large volumes of smoke and caused very bad fouling of the barrel whenever a shot was fired. To improve this condition a nitrocellulose powder was developed which reduced the smoke and fouling. This nitrocellulose powder was a great improvement over black powder but did not give perfect results because, although nitrocellulose does not 10 give the smoke or fouling attending black powder, there is a very noticeable flash attending each shot. It was desirable to completely eliminate the flash attending each shot. It was also desirable to produce powders which would be resis- 15 tant to moisture but the black powders and nitrocellulose powders were hygroscopic.

The ballistics which were obtained with the various nitrocellulose powders did not present major difficulties as it was possible to obtain the 20 desirable bullet velocities and breech pressures with comparative ease. But the performance of these powders with regard to flash, and smoke produced and their inability to resist moisture were serious handicaps to efficient operations and 25 uniform performance.

The problem of flash is a major problem to the ordnance art as the flash developed by a gun provides the enemy with a method of accurately locating the position of the piece. The flash is 30 easily noticeable by direct ground observation or by aerial reconnaissance, and results in enemy fire which may effectively destroy a battery of guns.

In a similar manner the smoke which is produced at each shot is objectionable since it allows the enemy to locate a battery of guns with comparative ease in daytime. The production of smoke upon firing a round is further disadvantageous because it obscures the vision of the gun crew 35 and prevents accurate firing.

In addition to preventing smoke and flashing the powder which is most desirable should also be non-hygroscopic as moisture adversely affects 40 the ballistics of the powder and results in non-uniform ranges for individual shots. Thus, there have been many attempts to produce a powder which will be smokeless, flashless, and non-hygroscopic while still giving the ballistics desired.

45 These three problems, flashing, smoke, and hy-

groscopicity, have resulted in a great deal of expensive research in attempting to find a method of producing a powder which is satisfactory for use in present day military operations.

There are at present a few smokeless powder 5 formulations which are classed as flashless and non-hygroscopic, but these powders, while the best known to the art, are not entirely satisfactory since they require the addition of two or more ingredients to the nitrocellulose to obtain 10 the proper ballistics and the desired flashlessness, smokelessness, and non-hygroscopicity. These types of powders are illustrated by U. S. Patent 1,854,776 which requires the addition of both an oxygen deficient and an oxygen carrying compound in the proper proportions to give the desired results. Such double additions are difficult to control, make the powder more expensive, and causes difficulties in obtaining the ballistics 15 desired.

20 The various powders now in use due to the variety of ingredients have higher charge weights for given ballistics than powders that do not contain ingredients for reducing flash, smoke and hygroscopicity. An economic problem is 25 thus introduced when attempting to produce a new powder that has the desired characteristics, due to the plurality of ingredients.

An object of this invention is to prepare a propellant powder which is smokeless, flashless, and 30 non-hygroscopic.

A further object of this invention is to produce a propellant powder for use in field pieces which 35 produces the desired ballistics without causing flashing.

A still further object of this invention is to produce a propellant powder which will give the desired ballistics with reduced charge weights.

Other objects will be apparent hereinafter. These objects may be accomplished in general 40 by colloidizing a mixture of nitrocellulose and dinitrotoluene, pressing the colloid into strands, and granulating to the desired grain size. The colloid may contain a small amount of diphenylamine or other equivalent compounds to act as 45 a stabilizer for the nitrocellulose.

Thus, in accordance with this invention, I have found that I may by using dinitrotoluene in conjunction with nitrocellulose produce a smokeless propellant powder that is flashless and non-hygroscopic. The percentage of dinitrotoluene which I use in my powder must be controlled in a very close range as I have found that less than about 21% of dinitrotoluene will allow the powder to flash while more than about 24% dinitro- 50 55

toluene causes the powder to produce undesired volumes of smoke. Therefore, the powder composition which I have found to be smokeless, flashless, and non-hygroscopic consists of an admixture of about 21% to about 24% dinitrotoluene and about 76% to about 79% nitrocellulose. This admixture will also contain about 1% by weight of a nitrocellulose stabilizer such as diphenylamine, the stabilizer which is normally added to all nitrocellulose powders to react with any decomposition products formed by the nitrocellulose in storage.

In manufacturing the powder of my invention, I have found that the nitrogen content of the nitrocellulose will affect the ballistics and hygroscopicity of the powder produced and I have found that the most desirable powder is produced when the nitrogen content of the nitrocellulose is above about 13% and preferably is about 13.2%.

Specific examples of the method of manufacturing the propellant powder of my invention and the results obtained by its use are as follows:

#### EXAMPLE 1

There were mixed in a Werner and Pfleiderer mixer 152 pounds of nitrocotton having an average nitrogen content of 13.21% with 46 pounds of 1, 2, 4, DNT, 2 pounds of diphenylamine, 47 pounds of alcohol and 43 pounds of acetone. This powder after proper mixing was blocked to cause further colloidizing and then pressed in the usual smokeless powder press through a die .140" in diameter and having seven perforation pins .020" in diameter. The strands of powder were cut into four pellets per inch by using a "Carney Point" cutting machine. After the cutting operation, the powder grains were water dried for 3 days at 50-55° C. and then air dried for 3 days at 55° C. The finished dried powder had a mean web of .0154 inch. Its hygroscopicity was 0.84% which is lower than that of most known powders. Hygroscopicity is determined by the standard U. S. Government methods. This improved powder made as above when tested in the 75 mm. gun model 1897 with a 12.37 pound projectile, and a 20.95 oz. charge gave a mean muzzle velocity of 1802 f. s. with 29,030 pounds per sq. in. pressure. After one year's storage at 50° C., the same charge of this powder gave identical velocity with a pressure of 29,660 pounds. No muzzle flash or smoke were observed in the test.

#### EXAMPLE 2

With 304 pounds of nitrocotton having an average nitrogen content of 13.22%, were mixed 92 pounds of 1, 2, 4, DNT, 4 pounds of diphenylamine, 70 pounds of alcohol, and 64 pounds of acetone. This powder was mixed in the usual manner, blocked, macaronied, reblocked, and pressed through a die .207" in diameter having 7 pins .018" in diameter and the resulting strand

cut into grains .4343" in length. This powder was given regular solvent recovery treatment for 2½ days at 55° C. then water dried 7 days at 55° C., and finally air dried for 2 days at 55° C. This powder had an average web of .03185". A test using a 7 lb. 9  $\frac{1}{16}$  oz. a full charge of this powder was made in the 155 mm. howitzer and gave an average muzzle velocity of 1459 f. s. with a pressure of 27,367 pounds.

#### EXAMPLE 3

There were mixed 39½ pounds dry weight of nitrocotton, 10 lbs. of liquid DNT, ½ lb. of diphenylamine, 10 lbs. of alcohol, 26 lbs. of ether, and 2½ lbs. of acetone in the usual W & P mixer and when the colloidizing was complete the powder mixture was pressed through a .085-.020 single pin die and the resulting strands cut four cuts to the inch. The powder grains were given five days water drying followed by three days air drying. There was no preliminary air drying or solvent recovery. This powder was tested in the 75 mm. model 1897 gun with the 11.72 lb. projectile with a charge of 20.6 ounces which gave a velocity of 1809 f. s. with 25,480 pounds pressure. This powder contains only 20% dinitrotoluene and the results were not satisfactory as the powder, when tested as described above while smokeless and non-hygroscopic, flashed in a number of the shots made.

#### EXAMPLE 4

Nitrocotton dry weight 152 lbs., liquid DNT 46 lbs., diphenylamine 2 lbs., alcohol 42 lbs., ether 35 lbs., and acetone 10 lbs. This powder was finished in exactly the same manner as in the previous example. When tested in the 75 mm. model 1897 under the same conditions as the previous example, this powder required 21 oz. to 40 give 1805 f. s. velocity with 24,100 lbs. pressure. No flash was noticed on any shot in tests which used a 16 oz. charge or a 21 oz. charge of powder.

In the above examples I have used as solvent the ether-alcohol, an ether-alcohol-acetone, or an alcohol-acetone mixture which is not usually accepted as possible in the manufacture of known single base smokeless powders.

From the above examples, it is noted that the powders produced are flashless, smokeless and non-hygroscopic and give the desired ballistics in the guns tested.

In order to show the superior performance of the powder of my invention, a comparison is given in the following table between the powder of this invention and a standard Government powder. It will be noted that when the charge weights are the same, the breech pressure is lower for the same velocity and when the pressures are kept constant, the velocity desired is obtained with a lower charge of powder.

TABLE 1  
155 mm. gun

| Test.....          | 1            | 2            | 3            | 4            | 5            | 6            | 7            | 8            |
|--------------------|--------------|--------------|--------------|--------------|--------------|--------------|--------------|--------------|
| 70 Projectile..... | 95 lb. slug. | 95 lb. slug. | 95 lb. slug. | 95 lb. slug. | 95 lb. slug. | 95 lb. slug. | 95 lb. slug. | 95 lb. slug. |
| Powder.....        | Powder #1.   | Powder #2.   | Powder #1.   | Powder #2.   | Powder #1.   | Powder #2.   | Powder #1.   | Powder #2.   |
| Charge.....        | 24.17 lbs... | 23.9 lbs...  | 24.17 lbs... | 24.78 lbs... | 24.17 lbs... | 24.18 lbs... | 24.17 lbs... | 24.6 lbs.    |
| Velocity.....      | 2,380        | 2,380        | 2,400        | 2,400        | 2,381        | 2,381        | 2,386        | 2,386        |
| Pressure.....      | 28,000       | 29,000       | 28,500       | 28,900       | 28,600       | 28,200       | 29,200       | 29,000       |

75 Powder #1—Government approved powder.  
Powder #2—Powder of my invention.

TABLE 2

## 155 mm. howitzer

| 5  | Test       | 1           | 2           | 3           | 4           | 5            | 6            | 5  |
|----|------------|-------------|-------------|-------------|-------------|--------------|--------------|----|
| 10 | Projectile | 95 lb. slug | 95 lb. slug | 95 lb. slug | 95 lb. slug | 95 lb. Mk. I | 95 lb. Mk. I |    |
|    | Powder     | Powder #1   | Powder #2   | Powder #1   | Powder #2   | Powder #1    | Powder #2    |    |
|    | Charge     | 8.1 lbs     | 7.9 lbs     | 8.1 lbs     | 7.76 lbs    | 8.16 lbs     | 8.10 lbs     |    |
|    | Velocity   | 1,484       | 1,484       | 1,476       | 1,485       | 1,471        | 1,471        | 10 |
|    | Pressure   | 26,700      | 28,200      | 27,800      | 29,500      | 29,200       | 28,700       |    |

Powder #1—Government approved powder.  
Powder #2—Powder of my invention.

15

TABLE 3

## 75 mm. pack howitzer

| 20 | Test       | 1               | 2               | 3               | 4               | 5               | 6               | 20 |
|----|------------|-----------------|-----------------|-----------------|-----------------|-----------------|-----------------|----|
| 25 | Projectile | 14.7 lb. Mk. II | 14.7 lb. Mk. II | 14.7 lb. Mk. II | 14.7 lb. Mk. II | 14.7 lb. Mk. II | 14.7 lb. Mk. II |    |
|    | Powder     | Powder #1       | Powder #2       | Powder #1       | Powder #2       | Powder #1       | Powder #2       |    |
|    | Charge     | 6.11 oz         | 5.8 oz          | 15.55 oz        | 14.7 oz         | 15.55 oz        | 13.9 oz         |    |
|    | Velocity   | 661             | 661             | 1,224           | 1,224           | 1,217           | 1,217           |    |
|    | Pressure   | 4,000           | 4,000           | 19,100          | 23,300          | 18,800          | 24,700          | 25 |

Powder #1—Government approved powder.  
Powder #2—Powder of my invention.

30

TABLE 4

## 105 mm. anti-aircraft

| 35 | Test       | 1           | 2           | 3           | 4           |  |
|----|------------|-------------|-------------|-------------|-------------|--|
| 40 | Projectile | 33 lb. slug | 33 lb. slug | 33 lb. slug | 33 lb. slug |  |
|    | Powder     | Powder #1   | Powder #2   | Powder #1   | Powder #2   |  |
|    | Charge     | 10.78 lbs   | 10.2 lbs    | 10.75 lbs   | 11.2 lbs    |  |
|    | Velocity   | 2,800       | 2,800       | 2,800       | 2,800       |  |
|    | Pressure   | 33,150      | 32,000      | 32,200      | 28,600      |  |

Powder #1—Government approved powder.  
Powder #2—Powder of my invention.

45

TABLE 5  
3" anti-aircraft

| 50 | Test       | 1             | 2             |  |
|----|------------|---------------|---------------|--|
| 55 | Projectile | 12.7 lb. slug | 12.7 lb. slug |  |
|    | Powder     | Powder #1     | Powder #2     |  |
|    | Charge     | 4.73 lbs      | 4.43 lbs      |  |
|    | Velocity   | 2,618         | 2,618         |  |
|    | Pressure   | 32,300        | 31,000        |  |

Powder #1—Government approved powder.  
Powder #2—Powder of my invention.

From the above tables the advantage of my powder in lower charge weight for desired ballistics when used in field pieces is brought out and also the advantage of maintaining low breech pressures with the same velocity is definitely shown. This powder further has the advantage of being economical to produce since there are only three ingredients necessary, to wit, nitrocellulose, dinitrotoluene and diphenylamine. In production, my powder is very easy to work, the pressing and cutting qualities being excellent. The cut grains are very smooth and regular and shrink in the normal manner to a uniform size. To show the improvement in hygroscopicity which is effected by the use of my powder, the results of tests on various samples are listed below in Table 6.

TABLE 6

| Powder            | Hygroscopicity |    |
|-------------------|----------------|----|
| Table 1—Test 4    | Percent        |    |
| Table 1—Test 6    | 0.71           | 35 |
| Table 2—Test 2    | 0.65           |    |
| Table 2—Test 4    | 0.81           |    |
| Table 3—Test 2    | 0.80           |    |
| Standard powders: | 0.84           |    |
| 1                 | 1.06           |    |
| 2                 | 1.07           |    |
| 3                 | 1.08           | 40 |

The powder is more economical than any of the known powders due to the reduced charges needed to obtain the desired ballistics, and due to the possibility of using alcohol-acetone mixtures as the solvent. The flashless, smokeless, and non-hygroscopic qualities are such that this powder has passed all ordnance tests.

It will be understood that the details and examples hereinbefore set forth are illustrative only, and that the invention as broadly described and claimed, is in no way limited thereby.

What I claim and desire to protect by Letters Patent is:

1. A propellant powder consisting essentially of nitrocellulose within the range of about 76% to about 79%, dinitrotoluene within the range of about 21% to about 24%, and diphenylamine within the range of about 0.8% to about 1.2%, said powder characterized by being smokeless and flashless.

2. A propellant powder consisting essentially of nitrocellulose within the range of about 76% to about 79%, dinitrotoluene within the range of about 21% to about 24%, and nitrocellulose stabilizer within the range of about 0.8% to about 1.2%, said powder characterized by being smokeless and flashless.

3. A propellant powder consisting essentially of nitrocellulose, having a nitrogen content of at least 13%, within the range of about 76% to about 79%, dinitrotoluene within the range of about 21% to about 24%, and diphenylamine within the range of about 0.8% to about 1.2%, 70 75

said powder characterized by being smokeless, flashless, and non-hygroscopic.

4. A propellant powder consisting essentially of nitrocellulose, having a nitrogen content of 5 at least 13%, about 77 parts by weight, dinitrotoluene about 23 parts by weight, and diphenylamine about 1 part by weight, said powder characterized by being smokeless, flashless, and non-hygroscopic.

10 5. A propellant powder consisting essentially of 77 parts by weight of nitrocellulose, 23 parts by weight of dinitrotoluene and 1 part by weight of diphenylamine.

6. A propellant powder consisting essentially

of 77 parts by weight of nitrocellulose having about 13.2% nitrogen content, 23 parts by weight of dinitrotoluene and 1 part by weight of diphenylamine.

7. A propellant powder consisting essentially of 5 nitrocellulose having a nitrogen content of at least 13%, within the range of about 76% to about 79%, dinitrotoluene within the range of about 21% to about 24%, and nitrocellulose stabilizer within the range of about 0.8% to about 1.2%, said powder characterized by being smokeless, flashless, and non-hygroscopic. 10

ELLSWORTH S. GOODYEAR.